

Patented Sept. 23, 1924.

1,509,172

# UNITED STATES PATENT OFFICE.

SIDNEY A. OGDEN, OF EAGLE ROCK, CALIFORNIA.

## PROCESS OF RECOVERING WOOL OR OTHER ANIMAL FIBERS FROM FABRICS.

No Drawing.

Application filed April 24, 1923. Serial No. 634,398.

To all whom it may concern:

Be it known that I, SIDNEY A. OGDEN, a subject of the King of Great Britain, residing at Eagle Rock, in the county of Los Angeles and State of California, have invented a certain new and useful Process of Recovering Wool or Other Animal Fibers from Fabrics, of which the following is a full, clear, and exact description.

10 The invention relates to the art of recovering wool, or other animal fibers from fabrics, whether the same be in the form of clothing or the like, or in the piece, in which the wool or hair may have been mixed with material such as cotton, and silk, during the process of manufacture.

It provides for a more complete recovery of valuable material in the so-called carbonizing process, inasmuch as the cotton may, 20 by the method proposed, be simultaneously or subsequently converted into the new and valuable substance termed hydro-cellulose, which is dehydrated hydro-cellulose in colloidal condition.

25 As the use of strong acids has an injurious effect on the wool, the present practice is to treat the woolen mixture with dilute acid, put into a drier, dust out the cotton (which is lost as useless by-product) and 30 treat the wool so reclaimed a second time, with water and a neutralizing substance.

35 By the method proposed, and hereinafter set forth, the two operations may, if desired, be combined, namely, the complete recovery of the wool unharmed, and the formation of hydro-cellulose, or hydro-cellulose derivatives.

40 This process of treating substances composed in part of wool is herein more particularly described, and a preferable manner of carrying it out will be hereinafter set forth:

Under my process, the woolen substances or articles are immersed in a strong acid, 45 preferably sulphuric acid of a Baumé concentration of about 50° to 58° and brought to a temperature of 50° to 70° centigrade. The length of time of immersion is governed by the strength of acid used and the temperature employed, but the best results for 50 commercial operations and economy are obtained by using strengths of about 50° Baumé with a temperature of about 70° centigrade.

55 Under these conditions, a rapid passing of the materials through the bath or im-

ersion effects an immediate disintegration of the cotton in a more or less colloidal state, which acts as a protecting influence to the wool by temporarily coating the wool 60 substance. The wool is then, as quickly as possible, passed into a washing bath to avoid any possibility of being damaged by the action of the acid.

An essential part of the process is therefore the speed in which the materials are passed through the acid bath. The affinity of the cellulose for the strong acid and the natural resistivity of the wool to liquids, permits the practicability of the process. 70 The cellulose material can then be recovered, or further treated to form dehydrated hydro-cellulose, and the wool dried by any convenient method after being washed free of acid.

75 Other methods with other acids of varying strengths may be used to separate the wool from the foreign material combined with it, but an important feature of this invention as set forth, is to protect the wool while effecting the separation, so the method used will not impair its quality.

It may be desirable in cases where there is insufficient material present in the woolen substance to form a protective coating on 85 the wool to saturate or cover the articles to be treated with a substance that will produce substantially the same effect. For instance, dipping the woolen articles to be treated in a thin cellulose paste or other protective substance is found to be advantageous, as the paste, or whatever substance is used when saturated with strong acid will 90 instantly destroy the fibers of the cotton upon contact, but will only superficially attack the wool.

95 That is to say it prevents the penetration of the acid into the woolen threads, and further damage whereto, by holding the acid in contact with the exterior surface only, and 100 which acid, as above mentioned, is removed before absorption can take place. On the other hand, the cotton or silk will absorb the strong acid and be instantly disintegrated.

105 The above process as outlined is equally suitable for the recovery of all such substances as animal fibers, etc., when admixed with foreign material.

110 A considerable advantage of this process, of further economic value, and which is practically unobtainable by other existing

processes, is the fact that the wool emerges from the wash bath in such a clean condition that the further operation known as "picking" can be eliminated, and should any foreign particles be unremoved they can be easily removed during the carding process.

Other advantages of the process consist in the production of a better grade of material, an increased volume of the production with lowered cost of production and overhead expenses, the elimination of hand-ripping, and the fact that no baking is required. It is moreover unnecessary to neutralize the acid, and furthermore the process eliminates the dust nuisance, and gas fumes, permits the recovery of wool from silk, and also the recovery of cotton as a valuable by-product. It furthermore permits the utilization of large quantities of waste, which are at present not recoverable.

It has been found in practice that if acids of required concentration to disintegrate with rapidity the foreign material mixed with the wool, and if the speed in which the acids are applied to the material to be treated is sufficiently increased, that the slower absorptive power of the wool or animal fibres prevent the penetration of the acid or acid fumes from having what would otherwise be, a harmful effect on the material treated.

It has been found that this process or method of treating woolen substances with strong sulphuric acid has a desirable effect on the fibres and a greatly improved material results.

These advantages have never been known before in the art of wool treatment, and are inseparable from the methods outlined for destroying foreign matter in admixture with wool by use of cellulose solvents or dispersing agents such as sulphuric acid.

Having thus described my invention, what I claim as new and desire to secure by Letters Patent of the United States is:

1. A process of treating material composed of wool and cellulose or silk in mechanical mixture whereby the wool can be reclaimed, and the additive substances or ma-

terials removed in such manner that valuable by-products may be recovered in the processing, without injury to the wool, which comprises causing protective substances to be formed on the woolen fibers before treating the whole for recovery of the by-products, and additive substances.

2. A process of treating material composed of animal fibers and cellulose or silk in mechanical mixture whereby the animal fibers may be reclaimed, and the additive substances or materials removed as a by-product recovered during the process without injury to the animal fibers, which comprises treating the animal fibers with an acid to convert the cellulose content to a hydro-cellulose known as colloidal hydro-cellulose in such a manner that until separation of the cellulose is effected a protecting coat of cellulose is formed on the animal fibers, recovering the by-products from the acid bath washing the animal fibers and drying the same.

3. A process of separating wool or similar animal fibers from the mixture thereof with vegetable fibers, which comprises passing said mixture rapidly through sulphuric acid at a concentration of about 50° Bé., at a temperature of approximately 65° C.

4. The process of separating wool or similar animal fibers from the mixture thereof with vegetable fibers, which comprises immersing the same a fraction of a minute in sulphuric acid at a concentration of about 50° Bé., at a temperature of approximately 65° C.

5. The process of separating wool or similar animal fibers from the mixture thereof with vegetable fibers, which comprises treating said mixture with sulphuric acid at a temperature between 50° and 70° C. at a concentration between 50° and 58° Bé. for such period of time as will dissolve or colloidalize vegetable matter such as cellulose but will not injure the animal fibers.

In testimony whereof I have hereunto set my hand this 24th day of April A. D. 1923.

SIDNEY A. OGDEN.